



US008808957B2

(12) **United States Patent**  
Hashimoto et al.

(10) **Patent No.:** US 8,808,957 B2  
(45) **Date of Patent:** Aug. 19, 2014

(54) **CARRIER FOR DEVELOPING ELECTROSTATIC IMAGE, DEVELOPER FOR ELECTROSTATIC IMAGE, DEVELOPING DEVICE, CARTRIDGE, PROCESS CARTRIDGE, IMAGE FORMING METHOD, AND IMAGE FORMING APPARATUS**

(75) Inventors: **Yasuaki Hashimoto**, Kanagawa (JP); **Yosuke Tsurumi**, Kanagawa (JP)

(73) Assignee: **Fuji Xerox Co., Ltd.**, Tokyo (JP)

(\*) Notice: Subject to any disclaimer, the term of this patent is extended or adjusted under 35 U.S.C. 154(b) by 326 days.

(21) Appl. No.: **13/091,807**

(22) Filed: **Apr. 21, 2011**

(65) **Prior Publication Data**

US 2012/0122028 A1 May 17, 2012

(30) **Foreign Application Priority Data**

Nov. 12, 2010 (JP) ..... 2010-253785

(51) **Int. Cl.**  
**G03G 9/00** (2006.01)

(52) **U.S. Cl.**  
USPC ..... 430/111.35; 430/111.1; 430/111.41;  
430/108.1

(58) **Field of Classification Search**

CPC ..... G03G 5/00; G03G 9/00  
USPC ..... 430/111.1, 11.35, 111.41, 108.1  
See application file for complete search history.

(56) **References Cited**

U.S. PATENT DOCUMENTS

5,223,366 A \* 6/1993 Kubo et al. ..... 430/111.1  
5,360,690 A \* 11/1994 Nakano et al. ..... 430/108.9

(Continued)

FOREIGN PATENT DOCUMENTS

JP A-8-171236 7/1996  
JP A-10-161355 6/1998

(Continued)  
OTHER PUBLICATIONS

English translation of JP 2005010183 A, Itami, Japan, Jan. 2005.\*

(Continued)

Primary Examiner — Mark F Huff

Assistant Examiner — Rashid Alam

(74) *Attorney, Agent, or Firm* — Oliff PLC

(57) **ABSTRACT**

A carrier for developing an electrostatic image, includes: magnetic core material particles and a coated layer coated on the magnetic core material particles, the coated layer containing a resin having a monomer unit represented by formula (A):



wherein R<sup>1</sup> represents a hydrogen atom or a methyl group; R<sup>2</sup> to R<sup>4</sup> each independently represent a hydrogen atom, an alkyl group, an aryl group or an aralkyl group; R<sup>5</sup> independently represents an alkyl group, an aryl group or an aralkyl group; n represents an integer of from 0 to 7; and L<sup>1</sup> represents a single bond or an alkylene group, provided that at least one of R<sup>3</sup> and R<sup>4</sup> is not a hydrogen atom.

**9 Claims, 1 Drawing Sheet**



(56)

**References Cited**

U.S. PATENT DOCUMENTS

5,932,387 A 8/1999 Yamamoto et al.  
2008/0085460 A1\* 4/2008 Ninomiya et al. .... 430/109.4  
2009/0109448 A1\* 4/2009 Kiyono et al. .... 358/1.1

FOREIGN PATENT DOCUMENTS

JP

A-10-307430 11/1998

JP

2005010183 A \* 1/2005

JP

A-2006-243236 9/2006

JP

A-2009-258477 11/2009

OTHER PUBLICATIONS

Arthur S. Diamond, Handbook of Imaging Materials, Nov. 28, 2001,  
Marcel Dekker, Inc., vol. 1, pp. 145-164.\*

\* cited by examiner



## 1

**CARRIER FOR DEVELOPING  
ELECTROSTATIC IMAGE, DEVELOPER FOR  
ELECTROSTATIC IMAGE, DEVELOPING  
DEVICE, CARTRIDGE, PROCESS  
CARTRIDGE, IMAGE FORMING METHOD,  
AND IMAGE FORMING APPARATUS**

CROSS-REFERENCE TO RELATED  
APPLICATIONS

This application is based on and claims priority under 35 USC 119 from Japanese Patent Application No. 2010-253785 filed Nov. 12, 2010.

BACKGROUND

1. Technical Field

The present invention relates to a carrier for developing an electrostatic image, a developer for an electrostatic image, a developing device, a cartridge, a process cartridge, an image forming method, and an image forming apparatus.

2. Related Art

A method of visualizing image information through an electrostatic latent image, such as an electrophotographic process, is being utilized in various fields of art. In the electrophotographic process, an electrostatic latent image is formed on a photoconductor through charging and exposing, and the electrostatic latent image is developed with a developer containing a toner and then visualized through transfer and fixing.

The developer used herein includes a two-component developer containing a toner and a carrier, and a single-component developer containing a toner solely, such as magnetic toner. The two-component toner is separated in functions of a developer, i.e., the carrier bears stirring, transportation and charging of the developer, thereby providing good controllability, and thus the two-component developer is being widely used. In particular, a developer containing a carrier having a resin coating is excellent in charge controlling property and thus may be relatively easily enhanced in environmental dependency.

SUMMARY

According to an aspect of the invention, there is provided a carrier for developing an electrostatic image, including: magnetic core material particles and a coated layer coated on the magnetic core material particles, the coated layer containing a resin having a monomer unit represented by following formula (A):



## 2

wherein R<sup>1</sup> represents a hydrogen atom or a methyl group; R<sup>2</sup> to R<sup>4</sup> each independently represent a hydrogen atom, an alkyl group, an aryl group or an aralkyl group; R<sup>5</sup> independently represents an alkyl group, an aryl group or an aralkyl group; n represents an integer of from 0 to 7; and L<sup>1</sup> represents a single bond or an alkylene group, provided that at least one of R<sup>3</sup> and R<sup>4</sup> is not a hydrogen atom.

BRIEF DESCRIPTION OF THE DRAWINGS

Exemplary embodiments of the present invention will be described in detail based on the following figures, wherein: FIG. 1 is a schematic illustration showing an example of an image output for evaluating image defect.

DETAILED DESCRIPTION

Exemplary embodiments of the invention will be described in detail below. The invention is not limited to the exemplary embodiments and may be practiced with various modifications unless the substance of the invention is impaired.

Carrier for developing Electrostatic Image

A carrier for developing an electrostatic image (which may be hereinafter referred simply to as a carrier) of the exemplary embodiment contains magnetic core material particles and a coated layer coated on the magnetic core material particles, and the coated layer contains a resin having a monomer unit represented by following formula (A):



wherein R<sup>1</sup> represents a hydrogen atom or a methyl group; R<sup>2</sup> to R<sup>4</sup> each independently represent a hydrogen atom, an alkyl group, an aryl group or an aralkyl group; R<sup>5</sup> independently represents an alkyl group, an aryl group or an aralkyl group; n represents an integer of from 0 to 7; and L<sup>1</sup> represents a single bond or an alkylene group, provided that at least one of R<sup>3</sup> and R<sup>4</sup> is not a hydrogen atom.

The inventors have found that the use of the resin having the monomer unit represented by the formula (A) is effective for enhancing the environmental dependency of the resin coated carrier.

The resin having the monomer unit represented by the formula (A) has such a structure that the nitrogen atoms of the piperidine rings are immobilized regularly aside the main chain, and the hydrocarbon group is present near the nitrogen atom of the piperidine ring, thereby decreasing the influence of water on the nitrogen atom. It is considered that owing to the structure, the developer using the carrier of the exemplary embodiment is stable in charging behavior irrespective of the environment, and the reproducibility of thin lines under a high

temperature and high humidity environment, which has been difficult to be achieved, is thus realized.

The constitutional components of the carrier will be described below.

#### Resin Coated Layer

The carrier of the exemplary embodiment has a coated layer coated on the magnetic core particles, and the coated layer contains a resin having a monomer unit represented by the formula (A), which may be hereinafter referred to as a particular resin. Examples of the resin having the monomer unit represented by the formula (A) include the following for enhancing the reproducibility of thin lines under a high temperature and high humidity.



(A)

wherein R<sup>1</sup> represents a hydrogen atom or a methyl group; R<sup>2</sup> to R<sup>4</sup> each independently represent a hydrogen atom, an alkyl group, an aryl group or an aralkyl group; R<sup>5</sup> independently represents an alkyl group, an aryl group or an aralkyl group; n represents an integer of from 0 to 7; and L<sup>1</sup> represents a single bond or an alkylene group, provided that at least one of R<sup>3</sup> and R<sup>4</sup> is not a hydrogen atom.

In the formula (A), R<sup>1</sup> may be a hydrogen atom. Accordingly, the monomer unit represented by the formula (A) may be a monomer unit derived from an acrylate compound.

In the formula (A), R<sup>2</sup> may be a hydrogen atom, an alkyl group or an aralkyl group, preferably a hydrogen atom or an alkyl group, more preferably a hydrogen atom or an alkyl group having from 1 to 4 carbon atoms, and further preferably a hydrogen atom or a methyl group.

In the formula (A), R<sup>3</sup> and R<sup>4</sup> each may independently represent a hydrogen atom or an alkyl group, preferably an alkyl group, more preferably an alkyl group having from 1 to 4 carbon atoms, and further preferably a methyl group, and still further preferably both R<sup>3</sup> and R<sup>4</sup> each represent a methyl group.

In the formula (A), at least one of R<sup>3</sup> and R<sup>4</sup> is not a hydrogen atom, and preferably both R<sup>3</sup> and R<sup>4</sup> are not a hydrogen atom.

In the formula (A), R<sup>5</sup>, which is a substituent on the piperidine ring, may be an alkyl group having from 1 to 8 carbon atoms, an aryl group having from 6 to 10 carbon atoms or an aralkyl group having from 7 to 18 carbon atoms, preferably an alkyl group having from 1 to 4 carbon atoms or a phenyl group, and more preferably a methyl group.

In the formula (A), n, which is the number of the substituent R<sup>5</sup>, may be from 0 to 4, preferably 2 or 3, and more preferably 2.

In the formula (A), L<sup>1</sup> may be a single bond or an alkylene group having from 1 to 4 carbon atoms, and more preferably a single bond.

In the formula (A), L<sup>1</sup> and R<sup>5</sup> are each bonded to an arbitrary position on the piperidine ring except for R<sup>2</sup> to R<sup>4</sup>, i.e., the positions shown by X on the piperidine ring shown in the following formula.

5



15

In the formula (A), may be bonded to any one of the 2 to 6-positions of the piperidine ring as described above, and is preferably bonded to the 4-position of the piperidine ring.

20

In the formula (A), R<sup>5</sup> is preferably bonded to at least one of the 2-position and the 6-position of the piperidine ring, and more preferably bonded to both the 2-position and the 6-position of the piperidine ring.

25

The monomer unit represented by the formula (A) is preferably a monomer unit represented by the following formula (A'), and more preferably a monomer unit represented by the following formula (A'').

(A')



(A'')



55

In the formulae (A') and (A''), R<sup>1</sup> represents a hydrogen atom or a methyl group; R<sup>2</sup> each independently represents a hydrogen atom, an alkyl group, an aryl group or an aralkyl group; R<sup>6</sup> represents an alkyl group; R<sup>7</sup> to R<sup>9</sup> each independently represent a hydrogen atom or an alkyl group; R<sup>10</sup> represents a hydrogen atom, an alkyl group, an aryl group or an aralkyl group; and L<sup>1</sup> represents a single bond or an alkylene group.

60

R<sup>1</sup>, R<sup>2</sup> and L<sup>1</sup> in the formula (A') and R<sup>1</sup> and R<sup>2</sup> in the formula (A'') have the same meanings as R<sup>1</sup>, R<sup>2</sup> and L<sup>1</sup> in the formula (A), respectively, and the exemplary ranges and the preferred ranges thereof are also the same.

In the formulae (A') and (A'') R<sup>6</sup> may be an alkyl group having from 1 to 4 carbon atoms, and preferably a methyl group.

In the formulae (A') and (A''), R<sup>7</sup> to R<sup>9</sup> each independently may be a hydrogen atom or an alkyl group having from 1 to 4 carbon atoms, preferably a hydrogen atom or a methyl group, and more preferably a methyl group.

In the formulae (A') and (A''), at least two of R<sup>7</sup> to R<sup>9</sup> each may be an alkyl group, preferably R<sup>7</sup> to R<sup>9</sup> are all alkyl groups, and more preferably R<sup>7</sup> to R<sup>9</sup> are all methyl groups.

In the formulae (A') and (A''), R<sup>10</sup> may be a hydrogen atom, an alkyl group or an aryl group, preferably a hydrogen atom or an aryl group, and more preferably a hydrogen atom.

Specific examples of the monomer unit represented by the formula (A) include monomer units represented by the following formulae (A-1) to (A-3).



(A-1)



(A-2)



(A-3)

Among these, the monomer units represented by the formulae (A-1) and (A-2) are preferred, and the monomer unit represented by the formula (A-2) is more preferred.

The resin having the monomer unit represented by the formula (A) may be a homopolymer or a copolymer.

The content of the monomer unit represented by the formula (A) may be approximately 10% by mol or more, preferably approximately 20% by mol or more, and more preferably approximately 30% by mol or more, based on the total monomer units of the resin having the monomer unit represented by the formula (A).

The synthesis method of the particular resin is not particularly limited, and for example, the resin may be synthesized by homopolymerization or copolymerization of a monomer represented by the following formula (M), or in alternative, synthesizing a resin having a monomer unit derived from acrylic acid or methacrylic acid, and then introducing the piperidine ring moiety thereto through polymer reaction. In consideration of easiness of synthesis and control of the structure of the resin, the resin may be synthesized by homopolymerization or copolymerization of a monomer represented by the following formula (M).



wherein R<sup>1</sup> represents a hydrogen atom or a methyl group; R<sup>2</sup> to R<sup>4</sup> each independently represent a hydrogen atom, an alkyl group, an aryl group or an aralkyl group; R<sup>5</sup> independently represents an alkyl group, an aryl group or an aralkyl group; n represents an integer of from 0 to 7; and L<sup>1</sup> represents a single bond or an alkylene group, provided that at least one of R<sup>3</sup> and R<sup>4</sup> is not a hydrogen atom.

R<sup>1</sup> to R<sup>5</sup>, n and L<sup>1</sup> in the formula (M) have the same meanings as R<sup>1</sup> to R<sup>5</sup>, n and L<sup>1</sup> in the formula (A), respectively, and the exemplary ranges and the preferred ranges thereof are also the same.

Specific examples of the monomer represented by the formula (M) include 2,2,6,6-tetramethyl-4-piperidyl acrylate, 1,2,2,6,6-pentamethyl-4-piperidyl acrylate, 1,2,5-trimethyl-4-phenyl-4-piperidyl acrylate, 2,2,6,6-tetramethyl-4-piperidyl methacrylate, 1,2,2,6,6-pentamethyl-4-piperidyl methacrylate, 1,2,5-trimethyl-4-phenyl-4-piperidyl methacrylate.

Examples of another monomer capable of being used for synthesizing the particular resin than the monomer represented by the formula (M) include an ethylenic unsaturated compound.

Specific examples of the ethylenic unsaturated compound include a styrene compound, such as styrene, p-chlorostyrene and  $\alpha$ -methylstyrene; an acrylate compound, such as methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, lauryl methacrylate and 2-ethylhexyl methacrylate; an unsaturated carboxylic acid, such as acrylic acid and methacrylic acid; an acrylonitrile compound, such as acrylonitrile and methacrylonitrile; a vinyl ether compound, such as vinyl ethyl ether and vinyl isobutyl ether; a ketone compound, such as vinyl methyl ketone, vinyl ethyl ketone and vinyl isopropenyl ketone; and an olefin compound, such as ethylene, propylene, butadiene and isoprene. Among these, a styrene compound and an acrylate compound are preferred.

The monomer may be used solely or as a combination of two or more kinds thereof.

The coated layer may contain carbon black. The carbon black contained may provide excellent suppression of image defect under a low temperature and low humidity environment.

The term "image defect" means such a phenomenon that a deletion due to thinning of the toner occurs at the tail end portion of the image, and it is considered that the image defect occurs in the following mechanism.

When a toner for developing an electrostatic image (which may be hereinafter referred simply to a toner) retained by a carrier is transferred to a photoconductor, the reverse charge with the polarity opposite to the charge of the toner is accumulated in the carrier. The reverse charge accumulated in the carrier attracts a part of the toner, which is thus attached again to the carrier. A deletion occurs consequently. The image defect tends to occur at the edge portion of the image that transits from a low density image to a high density image. In this case, the density at the tail end portion of the low density image is decreased. It is considered that the toner attached to the low density image portion is pulled back to the developer with the electric field in the high density image portion. In general, a resistance under a low temperature and low humidity environment is higher than a resistance under a high temperature and high humidity environment. When the difference in resistance therebetween is large, a carrier that is designed for the resistance under a high temperature and high humidity environment is too high in resistance under a low temperature and low humidity environment, and thus may cause the image defect.

The image defect tends to occur when the resistance of the carrier is higher since the charge therein is hard to erased, and it is therefore considered that the image defect may be suppressed from occurring by adding carbon black to the coated layer to lower the resistance of the carrier. Furthermore, it is considered that the electron distribution becomes homogeneous by the synergistic effect of the unshared electron pair of the nitrogen atom of the piperidine ring in the particular resin and the  $\pi$  electrons of the carbon black, and thus the addition of the carbon black suppresses the image defect from occurring.

The carbon black may have a volume average particle size of approximately 0.5  $\mu\text{m}$  or less, preferably from approximately 0.01  $\mu\text{m}$  to approximately 0.5  $\mu\text{m}$ , and more preferably from approximately 0.03  $\mu\text{m}$  to approximately 0.35  $\mu\text{m}$ . When the volume average particle size is in the range, the carbon black is hard to be dropped off from the coated layer, thereby providing stable charging property.

The volume average particle size of the carbon black may be measured with a laser diffraction particle size distribution measuring device (LA-700, available from Horiba, Ltd.).

The volume average particle size of the carbon black may be measured in such a manner that 2 g of a sample to be measured is put in 50 mL of a surfactant aqueous solution, which may be a 5% aqueous solution of sodium alkylbenzenesulfonate, and dispersed with an ultrasonic dispersing device (1,000 Hz) for 2 minutes to prepare a measurement sample, which is then measured.

The volume average particle sizes of each of the channels are accumulated from the small volume average particle size side, and the value at an accumulation of 50% is designated as the volume average particle size.

Examples of the carbon black include furnace black, ketchen black and channel black.

Specific examples thereof include #3350B, #30 and #3030B, available from Mitsubishi Chemical Corporation, #5500, available from Tokai Carbon Co., Ltd., granular acetylene black, available from Denki Kagaku Kogyo Kabushiki

Kaisha, HS-500, Asahi Thermal FT and Asahi Thermal MT, available from Asahi Carbon Co., Ltd., ketchen black, available from Lion Akzo Co., Ltd., Vulcan XC-72, Regal 400R and Monarch 1300, available from Cabot Specialty Chemicals, Inc., and Color Black FW200, Special Black 4, Printex 150T, Printex 140T and Printex U, available from Degussa AG.

The content of the carbon black in the coated layer may be 15.0% by weight or less, or approximately 15.0% by weight 10 or less, preferably from approximately 3.0 to 12.0% by weight, and more preferably from approximately 4.0 to 10.0% by weight, based on the total weight of the particular resin in the coated layer.

The resistance of the carrier may be necessarily high for 15 providing reproducibility of thin lines under a high temperature and high humidity environment. When the resistance of the carrier is low, the toner has low charging property, and the toner excessively developed on thin lines. When the content of the carbon black is in the range, excellent reproducibility of 20 thin lines under a high temperature and high humidity environment may be obtained.

The carrier of the exemplary embodiment may contain a charge controlling agent. The charge controlling agent may be used in combination with the carbon black.

25 The charge controlling agent may be any known charge controlling agent, such as a nigrosine dye, a benzimidazole compound, a quaternary ammonium salt compound, an alkoxyated amine, an alkylamide, a molybdcic acid chelate pigment, a triphenylmethane compound, a salicylic acid chelate compound, an azo-chromium complex and copper phthalocyanine. Preferred examples among these include a quaternary ammonium salt compound, an alkoxyated amine and an alkylamide.

30 The amount of the charge controlling agent added may be 35 from approximately 0.001 part by weight to approximately 5 parts by weight, and preferably from approximately 0.01 part by weight to approximately 0.5 part by weight, per 100 parts by weight of the particular resin in the coated layer. When the amount of the charge controlling agent is in the range, the 40 coated layer has a sufficient strength, which provides a carrier that is hard to be degraded due to stress upon use, and also provides good dispersibility of the electroconductive material.

The coated layer may also contain wax.

45 Wax is hydrophobic, and is relatively soft with low film strength at ordinary temperature. These are derived from the molecular structure of wax, and when the coated layer contains wax, such toner components as fine particles referred to as an external additive added to the surface of the toner and 50 toner bulk component are prevented from being attached to the surface of the carrier owing to the properties of wax. Furthermore, even when the toner components are attached to the surface of the carrier, the surface is renewed by flaking of the wax molecules from the attached part, thereby preventing 55 the surface of the carrier from being contaminated.

The wax is not particularly limited, and examples thereof include paraffin wax and a derivative thereof, montan wax and a derivative thereof, microcrystalline wax and a derivative thereof, Fischer-Tropsch wax and a derivative thereof, 60 and polyolefin wax and a derivative wax. The derivative referred herein includes a polymer with a vinyl monomer and a graft-modified product. Examples of the wax also include an alcohol, a fatty acid, vegetable wax, animal wax, mineral wax, ester wax and an acid amide. Any other known wax may be used.

65 The wax may have a melting point of from approximately 60° C. to approximately 200° C., and preferably from

approximately 80° C. to approximately 150° C. When the melting point of the wax is approximately 60° C. or more, the carrier may have excellent flowability.

The coated layer may contain another resin in addition to the particular resin.

Examples of the another resin used in the coated layer include polyethylene, polypropylene, polystyrene, polyacrylonitrile, polyvinyl acetate, polyvinyl alcohol, polyvinyl butyral, polyvinyl chloride, polyvinylcarbazole, polyvinyl ether, polyvinyl ketone, a vinyl chloride-vinyl acetate copolymer, a styrene-acrylic acid copolymer, a linear silicone resin containing an organosiloxane bond and a modified product thereof, a fluorine resin, polyester, polyurethane, polycarbonate, a phenol resin, an amino resin, a melamine resin, a benzoguanamine resin, a urea resin, an amide resin and an epoxy resin, but the another resin is not limited to the examples.

The coated layer may contain electroconductive powder other than carbon black.

Examples of the electroconductive powder include metal particles, such as gold, silver and copper; a semielectroconductive oxide particles, such as titanium oxide and zinc oxide; and particles containing powder, such as titanium oxide, zinc oxide, barium oxide, aluminum borate and potassium titanate, coated with tin oxide, a metal or the like.

The electroconductive powder may be used solely or as a combination of two or more kinds thereof.

The electroconductive powder may have a volume electric resistance of from approximately  $10^1 \Omega \cdot \text{cm}$  to approximately  $10^{11} \Omega \cdot \text{cm}$ , and preferably from approximately  $10^3 \Omega \cdot \text{cm}$  to approximately  $10^9 \Omega \cdot \text{cm}$ .

The volume electric resistance of the electroconductive powder may be measured in the same manner as the volume electric resistance of the core material particles described later.

The electroconductive powder may have a volume average particle size of approximately 0.5  $\mu\text{m}$  or less, preferably from approximately 0.05  $\mu\text{m}$  to approximately 0.5  $\mu\text{m}$ , and more preferably from approximately 0.05  $\mu\text{m}$  to approximately 0.35  $\mu\text{m}$ .

The content of the electroconductive powder is not particularly limited, and when the coated layer contains the carbon black, the content of the electroconductive powder may be smaller than the content of the carbon black.

The coated layer may contain resin particles.

Examples of the resin particles include thermoplastic resin particles and thermosetting resin particles. Among these, thermosetting resin particles are preferred since the hardness thereof may be increased relatively easily. The resin particles may be used solely or as a combination of two or more kinds thereof.

The resin particles may have a volume average particle size of from approximately 0.1  $\mu\text{m}$  to approximately 2.0  $\mu\text{m}$ , and preferably from approximately 0.2  $\mu\text{m}$  to approximately 1.0  $\mu\text{m}$ .

The content of the resin particles is not particularly limited, and when the coated layer contains the carbon black, the content of the resin particles may be smaller than the content of the carbon black.

The coated layer may contain known additives depending on necessity.

The method for forming the coated layer on the surface of the core material particles is not particularly limited, and examples of the method include a method of using a coating composition for forming a coated layer containing the particular resin and optional components, such as the carbon black and the charge controlling agent, in a solvent.

Examples of the method include a dipping method of dipping the core material particles in the coating composition for forming the coated layer, a spraying method of spraying the coating composition on the surface of the core material particles, and a kneader-coater method of mixing the core material particles and the coating composition, and then removing the solvent, in the state where the core material particles are floated with air flow. Among these, a kneader-coater method may be preferred in the exemplary embodiment.

The solvent used in the coating composition for forming a coated layer is not particularly limited and may be any one that dissolves only the resin, and the solvent may be selected from known solvents. Specific examples thereof include an aromatic hydrocarbon compound, such as toluene and xylene, a ketone compound, such as acetone and methyl ethyl ketone, and an ether compound, such as tetrahydrofuran and dioxane.

The coated layer is not limited to a single layer and may have a structure containing two or more layers.

The total content of the coated layer in the carrier of the exemplary embodiment may be from approximately 0.5 part by weight to approximately 10 parts by weight, preferably from approximately 1 part by weight to approximately 5 parts by weight, and more preferably from approximately 1 part by weight to approximately 3 parts by weight, per 100 parts by weight of the core material particles. When the content of the coated layer is approximately 0.5 part by weight or more, the surface of the core material powder is less exposed, and injection of the developing electric field is prevented. When the content of the coated layer is approximately 10 parts by weight or less, the coated layer forms a less amount of resin powder released therefrom, and the formation of resin powder due to release off during development may be prevented from the initial stage.

The coverage of the coated layer on the surface of the core material particles in the carrier of the exemplary embodiment may be approximately 80% or more, and preferably approximately 85% or more, and may be preferably as close as possible to 100%, while depending on the surface shape of the core material particles. When the coverage is approximately 80% or more, a deletion on an image may be suppressed from occurring.

Examples of a method for measuring the coverage of the coated layer in the carrier of the exemplary embodiment include a method of observing with an optical microscope, and a method of measuring by XPS measurement shown below.

In the XPS measurement, for example, an XPS measurement device may be JPS 80, available from JEOL, Ltd., and the measurement may be performed for the major element constituting the coated layer (which is generally carbon) and the major element constituting the core material particles

(which is generally iron and oxygen when the core material particles are constituted by an iron oxide series material, such as magnetite) with MgK $\alpha$  line as the X-ray source at an acceleration voltage of 10 kV and an emission current of 20 mV. (In the following description, the case where the core material particles are constituted by an iron oxide series material will be described.) The C 1s spectrum is measured for carbon, the Fe 2p<sub>3/2</sub> spectrum is measured for iron, and O 1s spectrum is measured for oxygen.

The number of atoms of carbon, oxygen and iron ( $A_c + A_o + A_{Fe}$ ) is obtained from the spectra of these elements. The iron amount of the core material particles and the iron amount of the carrier containing the core material particles coated with

## 11

the coated layer are obtained according to the following expression (9), and the coverage is obtained according to the expression (10).

$$\text{iron amount (atomic %)} = (A_{Fe}/(A_c+A_o+A_{Fe})) \times 100 \quad (9)$$

$$\text{coverage (\%)} = (1 - (\text{iron amount of carrier})/(\text{iron amount of core material particles})) \times 100 \quad (10)$$

In the case where a material other than the iron oxide series material is used as the core material particles, the coverage may be obtained in such a manner that the spectrum of a metal element constituting the core material particles is measured in addition to oxygen, and the similar calculation may be performed according to the expressions (9) and (10).

The coated layer may have an average thickness of from approximately 0.1  $\mu\text{m}$  to approximately 10  $\mu\text{m}$ , preferably from approximately 0.1  $\mu\text{m}$  to approximately 3.0  $\mu\text{m}$ , and more preferably from approximately 0.1  $\mu\text{m}$  to approximately 1.0  $\mu\text{m}$ .

The average thickness ( $\mu\text{m}$ ) of the coated layer may be obtained according to the following expression (11) from the true specific gravity  $\rho$  (dimensionless) of the core material particles, the volume average particle size  $d$  ( $\mu\text{m}$ ) of the core material particles, the average specific gravity  $\rho_c$  of the coated layer, and the total content  $W_c$  (part by weight) of the coated layer per 100 parts by weight of the core material particles.

$$\begin{aligned} \text{average thickness } (\mu\text{m}) &= ((\text{coated amount per one carrier particle}) \\ &\quad (\text{including additives, such as electroconductive powder})/ \\ &\quad (\text{surface area of one carrier particle})) \\ &\quad (\text{average specific gravity of coated layer}) = \\ &= (((4/3) \cdot \pi \cdot (d/2)^3 \cdot \rho \cdot W_c) / (4\pi \cdot (d/2)^2)) / \rho_c = \\ &= (1/6) \cdot (d \cdot \rho \cdot W_c / \rho_c) \end{aligned} \quad (11)$$

## Magnetic Core Material Particles

Examples of the magnetic core material particles (which may be hereinafter referred simply to as a core material) used in the carrier of the exemplary embodiment include resin particles having a magnetic metal, a magnetic oxide or magnetic particles dispersed therein.

The material of the magnetic particles (core material) used in the carrier of the exemplary embodiment is not particularly limited as far as the material satisfies the following conditions.

Specific examples thereof include a magnetic metal, such as iron, steel, nickel and cobalt, an alloy of the magnetic metal and another metal, such as manganese, chromium and a rare earth element, and a magnetic oxide, such as ferrite and magnetite.

Preferred examples of the core material include ferrite particles since a uniform surface and stable charging property may be obtained.

Examples of the ferrite for the core material include the following ferrite materials.



wherein M represents at least one selected from Cu, Zn, Fe, Mg, Mn, Ca, Li, Ti, Ni, Sn, Sr, Al, Ba, Co, Mo and the like, and X and Y each represent the proportion in terms of molar ratio, provided that  $X+Y=100$ .

Such a ferrite material may be preferred that M is one of or a combination of plural kinds of Li, Mg, Ca, Mn, Sr and Sn, and the content of the other component than M is approxi-

## 12

mately 1% by weight or less. When the aforementioned metal elements are contained, the core material may have a suitable electric resistance, the coverage may be easily controlled to an intended range, and excellent environmental dependency may be obtained.

Among these, M is preferably one of or a combination of plural kinds of Li, Mn, Mg and Sr. When Li is contained, the resistance is hard to be broken down upon application of a strong electric field. When Mn is contained, a high saturated magnetization may be obtained. When Mg is contained, the specific gravity may be decreased. When Sr is contained, the saturated magnetization may be increased. Thus, these elements are preferred as the magnetic core material.

The core material may be formed through granulation and baking, and as a pre-treatment, the core material may be finely pulverized. The pulverizing method is not particularly limited, and known pulverizing methods may be employed. Examples of the pulverizing method include methods using a mortar, a ball mill and a jet mill. The final pulverized state after the pre-treatment varies depending on the material and the like, and the volume average particle size of the core material before granulation and baking may be from approximately 2  $\mu\text{m}$  to approximately 10  $\mu\text{m}$ . When the volume average particle size is in the range, the material may have a particle size that is suitable for use, and an intended particle size may be easily obtained with an appropriate circularity.

The core material used in the exemplary embodiment may be resin particles having magnetic particles dispersed therein (which may be hereinafter referred to as magnetic material dispersed resin particles).

Examples of the magnetic material dispersed in the core material include a magnetic metal, such as iron, steel, nickel and cobalt; an alloy of the magnetic metal and another metal, such as manganese, chromium and a rare earth element (e.g., nickel-iron alloy, aluminum-iron alloy); and a magnetic oxide, such as ferrite and magnetite. Among these, iron oxide is preferred. Iron oxide particles as the magnetic material particles are stable and less toxic.

The magnetic material may be used solely or as a combination of two or more kinds thereof.

The magnetic material may have a volume average particle size of from approximately 0.01  $\mu\text{m}$  to approximately 1  $\mu\text{m}$ , preferably from approximately 0.03  $\mu\text{m}$  to approximately 0.5  $\mu\text{m}$ , and more preferably from approximately 0.05  $\mu\text{m}$  to approximately 0.35  $\mu\text{m}$ . When the volume average particle size of the magnetic material is in the range, sufficient saturation magnetization or suitable viscosity of the composition (monomer mixture) is obtained to provide a carrier with a uniform particle size and uniform magnetic material dispersed resin particles.

The content of the magnetic material in the magnetic material dispersed resin particles may be from approximately 30% by weight to approximately 99% by weight, preferably from approximately 45% by weight to approximately 97% by weight, and more preferably from approximately 60% by weight to approximately 95% by weight. When the content of the magnetic material is in the range, the carrier containing the magnetic material dispersed resin particles as a core material (i.e., a magnetic material dispersed carrier) is less scattered, and a magnetic brush of the magnetic material dispersed carrier does not become too hard to prevent the brush from being broken.

Examples of the resin component in the magnetic material dispersed resin particles include a cross linked styrene resin, an acrylic resin, a styrene-acrylic copolymer resin and a phenol resin.

## 13

The magnetic material dispersed resin particles used in the exemplary embodiment may further contain, in addition to the resin component and the magnetic material powder, other components depending on purposes. Examples of the other components include a charge controlling agent and fluorine-containing particles.

Examples of the preparation method of the magnetic material dispersed resin particles include a melt-kneading method, in which the magnetic material powder and the binder resin, such as a styrene-acrylic resin, are melt-kneaded with a Banbury mixer, a kneader or the like, and then cooled, followed by pulverization and classification (as described, for example, in JP-B-59-24416 and JP-B-8-3679), a suspension polymerization method, in which a monomer of the binder resin and the magnetic material powder are dispersed in a solvent to prepare a suspension liquid, and the suspension liquid is subjected to polymerization (as described, for example, in JP-A-5-100493), and a spray drying method, in which the magnetic material powder is mixed and dispersed in a solution of the resin, and the solution is spray-dried.

The core material may have a volume average particle size of from approximately 10  $\mu\text{m}$  to approximately 500  $\mu\text{m}$ , preferably from approximately 20  $\mu\text{m}$  to approximately 150  $\mu\text{m}$ , and more preferably from approximately 30  $\mu\text{m}$  to approximately 100  $\mu\text{m}$ . When the volume average particle size of the core material is approximately 10  $\mu\text{m}$  or more, the adhesion force between the toner and the carrier upon using for developing an electrostatic image may be appropriate to provide a sufficient developed amount of the toner. When the volume average particle size thereof is approximately 500  $\mu\text{m}$  or less, the magnetic brush may not be coarse to provide a fine image.

The volume average particle size of the core material may be measured, for example, with Coulter Counter TA-II (available from Beckman Coulter, Inc.), Coulter Multisizer II (available from Beckman Coulter, Inc.), a laser diffraction/scattering particle size analyzer (LS Particle Size Analyzer LS13, 320, available from Beckman Coulter, Inc.) and the like. The volume average particle sizes of each of the channels are accumulated from the small volume average particle size side, and the value at an accumulation of 50% is designated as the volume average particle size.

The carrier may have a weight average particle size of from approximately 15  $\mu\text{m}$  to approximately 500  $\mu\text{m}$ , and preferably from approximately 25  $\mu\text{m}$  to approximately 150  $\mu\text{m}$ . When the volume average particle size of the carrier is approximately 15  $\mu\text{m}$  or more, the carrier may be less contaminated. When the volume average particle size of the carrier is approximately 500  $\mu\text{m}$  or less, deterioration of the toner on stirring may be prevented.

The volume average particle size of the carrier may be measured, for example, with Coulter Counter TA-II (available from Beckman Coulter, Inc.), Coulter Multisizer II (available from Beckman Coulter, Inc.), a laser diffraction/scattering particle size analyzer (LS Particle Size Analyzer LS13, 320, available from Beckman Coulter, Inc.) and the like.

The carrier may have a shape factor SF1 of from approximately 100 to approximately 145 for achieving both high image quality and stirring efficiency of the developer.

The shape factor SF1 of the carrier means a value obtained by the following expression (12).

$$SF1 = 100\pi \times (ML)^2 / (4 \times A) \quad (12)$$

wherein ML represents the maximum length of the carrier particles, and A represents the projected area of the carrier particles.

## 14

The maximum length and the projected area of the carrier particles may be measured in such a manner that the carrier particles sampled on slide glass are observed with an optical microscope, and the image is input for image analysis to an image analyzer (Luzex III, available from Nireco Corporation) through a video camera. The number of the sampled carrier particles is 100 or more, and the shape factor SF1 is calculated by using the average value of the sampled carrier particles according to the expression (12).

## 10 Developer for Electrostatic Image

The developer for an electrostatic image (which may be hereinafter referred to as a developer) of the exemplary embodiment is a two-component developer, which may contain a carrier for developing an electrostatic image according to the exemplary embodiment and a toner for developing an electrostatic image.

The mixing ration (weight ratio) of the carrier for developing an electrostatic image of the exemplary embodiment and a toner for developing an electrostatic image in the developer 20 for an electrostatic image of the exemplary embodiment (toner/carrier) may be from approximately 1/99 to approximately 20/80, and preferably from approximately 3/97 to approximately 12/88.

The mixing method of the carrier and the toner is not 25 particularly limited, and they may be mixed with known apparatus and method, such as a V-blender.

## Toner for Developing Electrostatic Image

The toner for developing an electrostatic image (which may be hereinafter referred to as a toner) used in the exemplary embodiment is not particularly defined and is not particularly limited as a toner, and a known toner may be used. Examples of the toner include a color toner containing a binder resin and a colorant. Examples of the toner also include an infrared ray absorbing toner containing a binder resin and an infrared ray absorbent.

## 35 Toner Mother Particles

Toner mother particles of the toner used in the exemplary embodiment may contain a binder resin and a colorant, and may further contain depending on necessity a releasing agent, 40 silica and a charge controlling agent.

Examples of the binder resin include homopolymers and copolymers of a styrene compound, such as styrene and chlorostyrene; a monoolefin compound, such as ethylene, propylene, butylene and isoprene; a vinyl ester compound, such as 45 vinyl acetate, vinyl propionate, vinyl benzoate and vinyl lactate; an  $\alpha$ -methylene aliphatic monocarboxylate ester compound, such as methyl acrylate, ethyl acrylate, butyl acrylate, dodecyl acrylate, octyl acrylate, phenyl acrylate, methyl methacrylate, ethyl methacrylate, butyl methacrylate and 50 dodecyl methacrylate; a vinyl ether compound, such as vinyl methyl ether, vinyl ethyl ether and vinyl butyl ether; a vinyl ketone compound, such as vinyl methyl ketone, vinyl hexyl ketone and vinyl isopropenyl ketone; and the like.

Representative examples of the binder resin include poly-55 styrene, a styrene-alkyl acrylate copolymer, a styrene-alkyl methacrylate copolymer, a styrene-acrylonitrile copolymer, a styrene-butadiene copolymer, a styrene-maleic anhydride copolymer, polyethylene and polypropylene. Examples of the binder resin further include polyester, polyurethane, an 60 epoxy resin, a silicone resin, polyamide, modified rosin and paraffin wax. Among these, a styrene-alkyl acrylate copolymer, a styrene-alkyl methacrylate copolymer and a polyester resin are preferred.

The binder resin used in the toner is not limited to an amorphous resin, but a crystalline resin may be used depending on necessity. The crystalline resin is not particularly limited as far as it has crystallinity, and examples thereof include

15

a crystalline polyester resin and a crystalline vinyl resin. From the standpoint of reproducibility of thin lines under a high temperature and high humidity environment, a crystalline polyester resin is preferred, and a crystalline aliphatic polyester resin having a suitable melting point is more preferred.

Examples of the colorant of the toner include magnetic powder, such as magnetite and ferrite, pigments, such as carbon black, lamp black, Chrome Yellow, Hansa Yellow, Benzidine Yellow, Indanthrene Yellow, Quinoline Yellow, Permanent Orange GTR, Pyrazolone Orange, Vulkan Orange, Watchyoung Red, Permanent Red, Brilliant Carmine 3B, Brilliant Carmine 6B, Du Pont Oil Red, Pyrazolone Red, Lithol, Rhodamine B Lake, Lake Red C, Rose Bengal, Aniline Blue, Ultramarine Blue, Calco Oil Blue, Methylene Blue Chloride, Phthalocyanine Blue, Phthalocyanine Green and Malachite Green Oxalate, and dyes, such as an acridine series, a xanthene series, an azo series, a benzoquinone series, an azine series, an anthraquinone series, a thioindigo series, a dioxadine series, a thiazine series, an azomethine series, an indigo series, a phthalocyanine series, an aniline black series, a polymethine series, a triphenylmethane series, a diphenylmethane series, a thiazine series, and a thiazole series, which may be used solely or as a combination of two or more kinds thereof.

Examples of the colorant also include C.I. Pigment Red 48:1, C.I. Pigment Red 122, C.I. Pigment Red 57:1, C.I. Pigment Yellow 97, C.I. Pigment Yellow 17, C.I. Pigment Blue 15:1 and C.I. Pigment Blue 15:3.

The content of the colorant in the toner may be from approximately 1 part by weight to approximately 30 parts by weight per 100 parts by weight of the binder resin of the toner. A colorant having been surface-treated and a pigment dispersant may also be used depending on necessity. A yellow toner, a magenta toner, a cyan toner, a black toner and the like may be prepared by appropriately selecting the colorants.

The toner may contain a releasing agent and a charge controlling agent depending on necessity.

Examples of the releasing agent include a low molecular weight polyolefin, such as polyethylene, polypropylene and polybutene; a silicone compound having a softening point on heating; a fatty acid amide compound, such as oleic acid amide, erucic acid amide, ricinoleic acid amide and stearic acid amide; vegetable wax, such as ester wax, carnauba wax, rice wax, candelilla wax, wood wax and jojoba oil; animal wax, such as beeswax; mineral wax, such as montan wax, ozokerite, ceresin, paraffin wax, microcrystalline wax and Fischer-Tropsch wax; petroleum wax; modified products thereof.

The amount of the releasing agent added may be approximately 50% by weight or less based on the total weight of the toner.

The charge controlling agent may be a known one and examples thereof include an azo metal complex compound, a metal complex compound of salicylic acid, and a charge controlling agent containing a resin having a polar group.

Examples of the preparation method of the toner mother particles include: a kneading and pulverizing method, in which a binder resin and a colorant, and depending on necessity a releasing agent, a charge controlling agent and the like are kneaded, pulverized and classified; a method, in which particles obtained by the kneading and pulverizing method are changed in shape thereof with mechanical impact or heat energy; an emulsification and aggregation method, in which a dispersion containing a binder resin emulsified dispersed therein and dispersions of a colorant and depending on necessity a dispersion of a releasing agent, a charge controlling

16

agent and the like are mixed, and the particles are aggregated and integrated by heating, thereby providing toner particles; an emulsion polymerization and aggregation method, in which a polymerizable monomer of a binder resin is emulsion-polymerized, and the dispersion and dispersions of a colorant and depending on necessity a releasing agent, a charge controlling agent and the like are mixed, and the particles are aggregated and integrated by heating, thereby providing toner particles; a suspension polymerization method, in which a polymerizable monomer of a binder resin and solutions of a colorant and depending on necessity a releasing agent, a charge controlling agent and the like are suspended in an aqueous solvent and then polymerized; and a dissolution and suspension method, in which a solution of a binder resin and a colorant, and depending on necessity a releasing agent, a charge controlling agent and the like is suspended in an aqueous solvent and granulated. Such a preparation method may also be employed that the toner mother particles obtained by the aforementioned methods are used as core particles, on which aggregated particles are attached and integrated by heating, thereby providing a core-shell structure.

Among these, the toner of the exemplary embodiment may be a toner prepared by the emulsification and aggregation method or the emulsion polymerization and aggregation method, i.e., an emulsion aggregation toner.

The toner mother particles thus prepared may have a volume average particle size of from approximately 2  $\mu\text{m}$  to approximately 8  $\mu\text{m}$ , and preferably from approximately 3  $\mu\text{m}$  to approximately 7  $\mu\text{m}$ .

The toner mother particles may have a pseudo-spherical shape from the standpoint of enhancement of the developing property, the transferring efficiency and the image quality. The sphericity of the toner mother particles may be expressed by the shape factor SF1 shown by the following expression (1), and the average value of the shape factor SF1 (average shape factor) of the toner mother particles used in the exemplary embodiment may be less than approximately 145, preferably approximately 115 or more and less than approximately 140, and more preferably approximately 120 or more and less than approximately 140. When the average value of the shape factor SF1 is less than approximately 145, good transferring efficiency may be obtained to provide high image quality.

$$SF1 = \frac{(ML)^2}{A} \times \frac{\pi}{4} \times 100 \quad (1)$$

In the expression (1), ML represents the maximum length of the toner mother particles, and A represents the projected area of the toner mother particles.

The average value of the shape factor SF1 (average shape factor) may be measured in such a manner that an optical micrograph of 1,000 toner particles magnified 250 times is analyzed with an image analyzer (Luzex III, available from Nireco Corporation), values of the shape factor SF1 are obtained from the maximum length and the projected area, and the obtained values are averaged.

The toner mother particles used in the exemplary embodiment are not limited in preparation method thereof, and a known method may be used.

#### External Additive

The external additive of the toner of the exemplary embodiment is not particularly limited, and at least one thereof may be a small-size inorganic oxide having a volume average

primary particle size of from approximately 7 to approximately 40 nm that bears the powder fluidity, the charge control and the like. Examples of the small-size inorganic oxide include silica, alumina, an oxide of titanium (such as titanium oxide and metatitanic acid), calcium carbonate, magnesium carbonate, calcium phosphate and carbon black.

Among these, silica particles and titanium oxide particles are preferred.

The external additive may have a surface that has been subjected to a hydrophobic treatment in advance. The hydrophobic treatment may enhance the dispersibility. Examples of the hydrophobic treatment of the surface include treatments with dimethyldimethoxysilane, hexamethyldisilazane (HMDS), methyltrimethoxysilane, isobutyltrimethoxysilane and decyltrimethoxysilane.

In addition to the small-size inorganic oxide, a large-size inorganic oxide having a volume average particle size of from approximately 20 nm to approximately 300 nm may be added. Examples of the large-size inorganic oxide particles include fine particles of silica, titanium oxide, metatitanic acid, aluminum oxide, magnesium oxide, alumina, barium titanate, magnesium titanate, calcium titanate, strontium titanate, zinc oxide, chromium oxide, antimony trioxide, magnesium oxide and zirconium oxide. Among these, particles selected from silica, titanium oxide and metatitanic acid may be preferably used.

The amount of the small-size inorganic oxide added may be from approximately 0.5 part by weight to approximately 2.0 parts by weight per 100 parts by weight of the toner mother particles. In the case where the large-size inorganic oxide is added, the amount of the large-size inorganic oxide may be from approximately 1.0 part by weight to approximately 5.0 parts by weight per 100 parts by weight of the toner mother particles.

Lubricant particles may be used as an external additive.

Examples of the lubricant particles include a solid lubricant, such as graphite, molybdenum disulfide, talc, a fatty acid, a higher alcohol, an aliphatic alcohol and a fatty acid metal salt; a low molecular weight polyolefin, such as polypropylene, polyethylene and polybutene; a silicone compound having a softening point upon heating; a fatty acid amide compound, such as oleic acid amide, erucic acid amide, ricinoleic acid amide and stearic acid amide; vegetable wax, such as carnauba wax, rice wax, candelilla wax, wood wax and jojoba oil; animal wax, such as beeswax; mineral or petroleum wax, such as montan wax, ozokerite, ceresin, paraffin wax, microcrystalline wax and Fischer-Tropsch wax; and modified products thereof.

An abrasive may be used as the external additive.

The abrasive may be a known inorganic oxide. Examples thereof include cerium oxide, strontium titanate, magnesium oxide, alumina, silicon carbide, zinc oxide, silica, titanium oxide, boron nitrate, calcium pyrophosphate, zirconia, barium titanate, calcium titanate and calcium carbonate. A composite material thereof may be used.

The toner may be prepared, for example, by mixing the toner mother particles and the external additives with a Henschel mixer, a V-blender or the like. In the case where the toner mother particles are prepared by a wet process, the external additives may be added by a wet process.

The developer of the exemplary embodiment may be used as a developer that is contained in a developing unit (e.g., a developer container) and may also be used as a replenisher developer used in a trickle developing system described later. Developing Device, Cartridge, Process Cartridge, Image Forming Method, and Image Forming Apparatus

A cartridge of the exemplary embodiment will be described.

The cartridge of the exemplary embodiment contains the carrier for developing an electrostatic image of the exemplary embodiment, or contains the developer for an electrostatic image of the exemplary embodiment. The cartridge of the exemplary embodiment may be detachable to an image forming apparatus.

The use of the cartridge of the exemplary embodiment containing the developer of the exemplary embodiment in an image forming apparatus or an image forming method may achieve both reproducibility of thin lines under a high temperature and high humidity environment and suppression of image defect under a low temperature and low humidity environment simultaneously.

The cartridge of the exemplary embodiment may be used in a developing device, an image forming method and an image forming apparatus, which has a trickle developing system.

In the case where the cartridge of the exemplary embodiment is used in a developing device, an image forming method or an image forming apparatus, the cartridge of the exemplary embodiment may contain the developer of the exemplary embodiment, or in alternative, the cartridge of the exemplary embodiment may contain the carrier of the exemplary embodiment solely, which may be used in combination with another cartridge containing a toner solely.

The image forming method of the exemplary embodiment may contain: charging an image holding member; exposing a surface of the image holding member, thereby forming an electrostatic latent image; developing the electrostatic latent image formed on the surface of the image holding member, with a two-component developer, thereby forming a toner image; transferring the toner image formed on the surface of the image holding member, to a surface of a transfer material; and fixing the toner image transferred to the transfer material, in which the two-component developer is the developer for an electrostatic image of the exemplary embodiment.

In the image forming method of the exemplary embodiment, a duplicated image may be formed, for example, in such a manner that a developer is prepared by using the particular carrier, an electrostatic image is formed and developed with the developer by using an ordinary electrophotographic duplicator, and the obtained toner image is transferred to transfer paper and then fixed thereto with a heat roller fixing device having a heating roller set at a prescribed temperature.

The carrier for developing an electrostatic image of the exemplary embodiment may be used in an image forming method of an ordinary electrostatic image developing process (electrophotographic process). The image forming method of the exemplary embodiment may contain, for example, formation of an electrostatic latent image (charging and exposing), development, transferring, and cleaning. These processes themselves are ordinarily practiced in the field of art, and described, for example, in JP-A-56-40868, JP-A-49-91231 and the like. The image forming method of the exemplary embodiment may be practiced by using an ordinarily known image forming apparatus, such as a duplicator, a facsimile machine and the like.

60 In the charging, an image holding member is charged.  
In the exposing, an electrostatic latent image is formed on a surface of the image holding member.

In the development, the electrostatic latent image is developed with a developer layer on a developer holding member, thereby forming a toner image. The developer layer is not particularly limited as far as it contains the developer for an electrostatic image of the exemplary embodiment containing

a toner for developing an electrostatic image and the carrier for developing an electrostatic image of the exemplary embodiment.

In the transferring, the toner image is transferred to a transfer material. Examples of the transfer material in the transferring include an intermediate transfer material and a recording medium such as a paper.

In the fixing, the toner image transferred to the transfer paper is fixed, for example, with a heat roller fixing device having a heating roller set at a prescribed temperature, thereby forming a duplicated image.

In the cleaning, the developer for an electrostatic image remaining on the electrostatic latent image holding member is removed.

The image forming method of the exemplary embodiment may contain recycling. In the recycling, the toner for developing an electrostatic image that has been recovered in the cleaning is sent to the developer layer. The image forming method of the exemplary embodiment containing the recycling may be practiced by using an image forming apparatus, such as a duplicator and a facsimile machine, having a toner recycling system. The image forming method of the exemplary embodiment may be applied to a recycling system, in which the toner is recovered simultaneously development, and the cleaning is omitted.

The image forming apparatus of the exemplary embodiment contains: an image holding member; a charging unit that charges the image holding member; an exposing unit that exposes the charged image holding member, thereby forming an electrostatic latent image on the image holding member; a developing unit that develops the electrostatic latent image with a two-component developer, thereby forming a toner image; a transferring unit that transfers the toner image from the image holding member to a transfer material; and a fixing unit that fixes the toner image transferred to the transfer material, in which the two-component developer is the developer for an electrostatic image of the exemplary embodiment.

The image forming apparatus of the exemplary embodiment is not particularly limited as far as it contains the image holding member, the charging unit, the exposing unit, the developing unit and the transferring unit, and may further contain a cleaning unit, an erasing unit and the like.

In the transferring unit, the transferring operation may be performed twice or more by using an intermediate transfer material. Examples of the transfer material in the transferring unit include an intermediate transfer material and paper.

The developing unit may contain: a developer container that contains the developer of the exemplary embodiment; a developer supplying unit that supplies the developer to the developer container; and a developer discharging unit that discharges at least a part of the developer contained in the developer container, i.e., may have a trickle developing system.

The developer to be supplied to the developer container (i.e., a replenisher developer) may have a mixing weight ratio of the toner and the carrier (toner/carrier) of from approximately 2 or more, preferably 3 or more, and more preferably 5 or more.

In the case where a resin coated carrier that is liable to suffer flaking of the coated layer is used the trickle developing system, not only flaking of the coated layer of the developer that is originally contained in the developer container occurs, but also flaking of the coated layer of the developer that is fed from the developer supplying unit to the developer container also occurs. Thus, the influence of resin powder released from the carrier is larger as compared to the case the trickle developing system is not used.

By using the image forming apparatus of the exemplary embodiment using the developer of the exemplary embodiment, however, the coated layer of the developer of the exemplary embodiment is hard to be flaked. Therefore, even when the trickle developing system is employed, the aforementioned problem may not occur. Furthermore, the charge distribution of the toner is stabilized, and both the reproducibility of thin lines under a high temperature and high humidity environment and the suppression of image defect under a low temperature and low humidity environment are achieved simultaneously.

The constitutional components including the image holding member, the units and the like each may have the structure described for the process of the image forming method. The constitutional components each may be a known component. The image forming apparatus of the exemplary embodiment may contain other units, devices and the like in addition to the aforementioned structure. The image forming apparatus of the exemplary embodiment may have a plurality of the constitutional component.

The process cartridge of the exemplary embodiment contains at least a developing unit that develops an electrostatic latent image formed on an image holding member, with the developer for an electrostatic image of the exemplary embodiment, thereby forming a toner image. The process cartridge of the exemplary embodiment may be detachable to an image forming apparatus.

The process cartridge of the exemplary embodiment may further contain other members, such as an erasing unit, depending on necessity.

The use of the process cartridge of the exemplary embodiment containing the developer of the exemplary embodiment in an image forming apparatus may achieve stable image formation for a prolonged period of time with less environmental dependency, such as temperature and humidity, and less flaking of the coated layer.

## EXAMPLES

The invention will be described in more detail with reference to examples below, but the invention is not limited to the examples.

### Measurement Methods

#### Volume Average Particle Size of Toner Mother Particles

The volume average particle size of the toner mother particles is measured with Coulter Multisizer II (available from Beckman Coulter, Inc.). The electrolytic solution used is ISO-TON-II (available from Beckman Coulter, Inc.).

The measurement is performed in the following manner. From 0.5 mg to 50 mg of a sample is put in 2 mL of a surfactant aqueous solution, which may be a 5% aqueous solution of sodium alkylbenzenesulfonate, and the solution is added to from 100 mL to 150 mL of the electrolytic solution.

The electrolytic solution having the sample dispersed therein is subjected to a dispersion treatment for 1 minute with an ultrasonic dispersing device, and the particle size distribution of the particles having a particle size of from 2.0  $\mu\text{m}$  to 60  $\mu\text{m}$  is measured with Coulter Multisizer II using an aperture having an aperture size of 100  $\mu\text{m}$ . The number of particles to be measured is 50,000.

The particle size distribution thus measured is divided into particle size ranges (channels), and an accumulated distribution is drawn for weight or volume from the small size side.

The particle size at an accumulation of 50% is designated as a weight average particle size or a volume average particle size.

## Shape Factor

The shape factor SF1 is obtained by the following expression.

$$SF1 = 100\pi \times (ML)^2 / (4 \times A)$$

wherein ML represents the maximum length of the particles, and A represents the projected area of the particles. The maximum length and the projected area of the particles are measured in such a manner that the particles sampled on slide glass are observed with an optical microscope, and the image is input for image analysis to an image analyzer (Luzex III, available from Nireco Corporation) through a video camera. The number of the sampled carrier particles is 100, and the shape factor SF1 is calculated by using the average value of the sampled particles according to the above expression.

## Glass Transition Temperature of Toner Mother Particles

The glass transition temperature (Tg) of the toner mother particles is measured with a differential scanning calorimeter (DSC-50, available from Shimadzu Corporation) at a condition of a temperature increasing rate of 3° C. per minute, in which the temperature at the intersecting point of the base line and the extended line of the rising line in the endothermic region is designated as the glass transition temperature.

## Coating Composition 1

|                                                                                                                                                        |                     |
|--------------------------------------------------------------------------------------------------------------------------------------------------------|---------------------|
| Copolymer particles of methyl methacrylate and 2,2,6,6-tetramethyl-4-piperidyl acrylate (weight ratio: 80/20, weight average molecular weight: 70,000) | 100 parts by weight |
| Carbon black (VXC72, available from Cabot Speciality Chemicals, Inc.)                                                                                  | 5.0 parts by weight |
| Toluene (available from Wako Pure Chemical Industries, Ltd.)                                                                                           | 500 parts by weight |

The aforementioned components and glass beads (particle size: 1 mm, the same amount as toluene) are put in a sand mill, available from Kansai Paint Co., Ltd., and stirred at a rotation rate of 1,200 rpm for 30 minutes, thereby preparing a coating composition 1 having a solid content of 18%.

## Coating Composition 2

A coating composition 2 is prepared in the same manner as in Coating Composition 1 except that copolymer particles of methyl methacrylate and 1,2,2,6,6-pentamethyl-4-piperidyl acrylate (weight ratio: 80/20) is used instead of the copolymer particles of methyl methacrylate and 2,2,6,6-tetramethyl-4-piperidyl acrylate.

## Coating Composition 3

A coating composition 3 is prepared in the same manner as in Coating Composition 1 except that copolymer particles of methyl methacrylate and 1,2,5-trimethyl-4-phenyl-4-piperidyl acrylate (weight ratio: 80/20) is used instead of the copolymer particles of methyl methacrylate and 2,2,6,6-tetramethyl-4-piperidyl acrylate.

## Coating Composition 4

A coating composition 4 is prepared in the same manner as in Coating Composition 1 except that the carbon black is not used.

## Coating Composition 5

A coating composition 5 is prepared in the same manner as in Coating Composition 1 except that the amount of the carbon black is changed to 16 parts by weight.

## Coating Composition 6

A coating composition 6 is prepared in the same manner as in Coating Composition 1 except that the weight ratio of the

copolymer particles of methyl methacrylate and 2,2,6,6-tetramethyl-4-piperidyl acrylate is changed from 80/20 to 90/10.

## Coating Composition 7

5 A coating composition 7 is prepared in the same manner as in Coating Composition 1 except that the weight ratio of the copolymer particles of methyl methacrylate and 2,2,6,6-tetramethyl-4-piperidyl acrylate is changed from 80/20 to 70/30.

## 10 Coating Composition 8

A coating composition 8 is prepared in the same manner as in Coating Composition 1 except that homopolymer particles of methyl methacrylate is used instead of the copolymer particles of methyl methacrylate and 2,2,6,6-tetramethyl-4-piperidyl acrylate.

## Coating Composition 9

A coating composition 9 is prepared in the same manner as in Coating Composition 1 except that copolymer particles of methyl methacrylate and dimethyl amino acrylate (weight ratio: 80/20) is used instead of the copolymer particles of methyl methacrylate and 2,2,6,6-tetramethyl-4-piperidyl acrylate.

## Coating Composition 10

25 A coating composition 10 is prepared in the same manner as in Coating Composition 8 except that the carbon black is not used.

## Coating Composition 11

30 A coating composition 11 is prepared in the same manner as in Coating Composition 8 except that the amount of the carbon black is changed to 16 parts by weight.

## Carrier 1

|                                                                                                                        |                       |
|------------------------------------------------------------------------------------------------------------------------|-----------------------|
| Mn—Mg ferrite (DFC350, available from Dowa Mining Co., Ltd. volume average particle size: 35 $\mu\text{m}$ , SF1: 135) | 2,000 parts by weight |
| Coating composition 1                                                                                                  | 320 parts by weight   |

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8

## Carrier 6

A carrier 6 is prepared in the same manner as in the carrier 1 except that the coating composition 6 is used instead of the coating composition 1.

## Carrier 7

A carrier 7 is prepared in the same manner as in the carrier 1 except that the coating composition 7 is used instead of the coating composition 1.

## Carrier 8

A carrier 8 is prepared in the same manner as in the carrier 1 except that the coating composition 8 is used instead of the coating composition 1.

## Carrier 9

A carrier 9 is prepared in the same manner as in the carrier 1 except that the coating composition 9 is used instead of the coating composition 1.

## Carrier 10

A carrier 10 is prepared in the same manner as in the carrier 1 except that the coating composition 10 is used instead of the coating composition 1.

## Carrier 11

A carrier 11 is prepared in the same manner as in the carrier 1 except that the coating composition 11 is used instead of the coating composition 1.

## Colorant Dispersion 1

|                                                                                                                                       |                     |
|---------------------------------------------------------------------------------------------------------------------------------------|---------------------|
| Cyan pigment<br>(copper phthalocyanine, C.I. Pigment Blue 15:3,<br>available from Dainichiseika Colour &<br>Chemicals Mfg. Co., Ltd.) | 50 parts by weight  |
| Anionic surfactant<br>(Neogen SC, available from Dai-ichi Kogyo<br>Seiyaku Co., Ltd.)                                                 | 5 parts by weight   |
| Ion exchanged water                                                                                                                   | 200 parts by weight |

The aforementioned components are mixed and dispersed with Ultra-Turrax, available from IKA Works, Inc., for 5 minutes and then with an ultrasonic bath for 10 minutes, thereby providing a colorant dispersion 1 having a solid content of 21%.

## Releasing Agent Dispersion 1

|                                                                                       |                    |
|---------------------------------------------------------------------------------------|--------------------|
| Paraffin wax<br>(HNP-9, available from Nippon Seiro Co., Ltd.)                        | 19 parts by weight |
| Anionic surfactant<br>(Neogen SC, available from Dai-ichi Kogyo<br>Seiyaku Co., Ltd.) | 1 part by weight   |
| Ion exchanged water                                                                   | 80 parts by weight |

The aforementioned components are mixed in a heat resistant vessel, and the mixture is heated to 90° C. and stirred for 30 minutes. The molten liquid is taken out from the bottom of the vessel and sent to Gaulin Homogenizer. After performing the circulation operation corresponding to three passes under a pressure of 5 MPa, the pressure is increased to 35 MPa, and the circulation operation corresponding to three passes is performed. The obtained emulsion liquid is cooled to 40° C. or lower in the heat resistant vessel, thereby providing a releasing agent dispersion 1.

## Resin Particle Dispersion

## Oily Layer

|                                                                    |                    |
|--------------------------------------------------------------------|--------------------|
| Styrene<br>(available from Wako Pure Chemical Industries,<br>Ltd.) | 30 parts by weight |
|--------------------------------------------------------------------|--------------------|

-continued

|                                                                             |                     |
|-----------------------------------------------------------------------------|---------------------|
| n-Butyl acrylate<br>(available from Wako Pure Chemical Industries,<br>Ltd.) | 10 parts by weight  |
| β-Carboxyethyl acrylate<br>(available from Rhodia Nicca, Ltd.)              | 1.3 parts by weight |
| Dodecanethiol<br>(available from Wako Pure Chemical Industries,<br>Ltd.)    | 0.4 part by weight  |

|    |                                                                                            |
|----|--------------------------------------------------------------------------------------------|
| 10 | Aqueous Layer 1                                                                            |
| 15 | Ion exchanged water<br>Anionic surfactant<br>(Dowfax, available from Dow Chemical Company) |

|    |                                                                                                                                                                                   |
|----|-----------------------------------------------------------------------------------------------------------------------------------------------------------------------------------|
| 20 | Aqueous Layer 2                                                                                                                                                                   |
| 25 | Ion exchanged water<br>Anionic surfactant<br>(Dowfax, available from Dow Chemical Company)<br>Ammonium peroxodisulfate<br>(available from Wako Pure Chemical Industries,<br>Ltd.) |

The components of the oily layer and the components of the aqueous layer 1 are mixed by stirring in a flask to prepare a monomer emulsion liquid. The component of the aqueous layer are put in a reactor, the interior of which is then sufficiently substituted with nitrogen gas, and the reaction system is heated to 75° C. over an oil bath under stirring. The monomer emulsion liquid is added slowly dropwise to the reactor over 3 hours to perform emulsion polymerization. After completing the dropwise addition, the polymerization is continued at 75° C. and terminated after lapsing 3 hours.

The resin particles has a volume average particle size  $D_{50v}$  of 250 nm as measured with a laser diffraction particle size distribution measuring device (LA-700, available from Horiba, Ltd.) and a glass transition temperature of 52° C. as measured with a differential scanning calorimeter (DSC-50, available from Shimadzu Corporation) at a temperature increasing rate of 10° C. per minute. Thus, a resin particle dispersion having a volume average particle size of 250 nm, a solid content of 42% and a glass transition temperature of 52° C. is obtained.

## Toner 1

|    |                              |                     |
|----|------------------------------|---------------------|
| 50 | Resin particle dispersion    | 150 parts by weight |
|    | Colorant dispersion 1        | 30 parts by weight  |
|    | Releasing agent dispersion 1 | 40 parts by weight  |
|    | Polyaluminum chloride        | 0.4 part by weight  |

55 The aforementioned components are sufficiently mixed and dispersed with Ultra-Turrax, available from IKA Works, Inc., in a stainless steel flask, and then heated to 48° C. under stirring over a heating oil bath. After maintaining at 48° C. for 80 minutes, 70 parts by weight of the same resin particle dispersion as above is slowly added thereto.

Thereafter, the pH inside the system is controlled to 6.0 with a sodium hydroxide aqueous solution having a concentration of 0.5 mol/L, and the reaction mixture is heated to 97° C. and maintained for 3 hours under continuously stirring 65 with the stainless steel flask being sealed and the stirrer shaft being sealed with a magnetic seal. After completing the reaction, the reaction mixture is cooled at a temperature decreas-

ing rate of 1°C. per minute and then filtered. The solid content is sufficiently rinsed with ion exchanged water, and then collected by solid-liquid separation by Nutsche suction filtration. The solid content is again dispersed in 3,000 parts by weight of ion exchanged water at 40°C. and stirred and rinsed at 300 rpm for 15 minutes. The rinsing operation is repeated five times, and when the pH of the filtrate becomes 6.54 and the electroconductivity thereof becomes 6.5  $\mu$ S/cm, the solid content is collected by solid-liquid separation by Nutsche suction filtration with No. 5A filter paper. The solid content is continuously dried under vacuum for 12 hours to provide toner mother particles.

The toner mother particles has a volume average particle size  $D_{50v}$  of 6.2  $\mu$ m and a volume average particle size distribution index GSD<sub>v</sub> of 1.20, as measured with Coulter Counter TA-II (available from Beckman Coulter, Inc.). The shape of the mother particles is observed with Luzex image analyzer (available from Nireco Corporation), and as a result, the particles have a shape factor SF1 of 135, which shows a potato-like shape. The glass transition temperature of the toner mother particles is 52°C. To the toner mother particles, silica (SiO<sub>2</sub>) fine particles having an average primary particle size of 40 nm having been subjected to a surface hydrophobic treatment with hexamethyldisilazane (which may be herein-after abbreviated as HMDS) and metatitanic acid compound fine particles having an average primary particle size of 20 nm, which are a reaction product of metatitanic acid and isobutyltrimethoxysilane, are added to make a coverage of 40% with respect to the surface of the colored particles, followed by mixing with a Henschel mixer, thereby providing a toner.

#### Preparation of Amorphous Resin Particle Dispersion

|                                                                           |                    |
|---------------------------------------------------------------------------|--------------------|
| Ethylene glycol<br>(available from Wako Pure Chemical Industries, Ltd.)   | 50 parts by weight |
| Neopentyl glycol<br>(available from Wako Pure Chemical Industries, Ltd.)  | 65 parts by weight |
| Terephthalic acid<br>(available from Wako Pure Chemical Industries, Ltd.) | 96 parts by weight |

The aforementioned monomers are charged in a flask, and the mixture is heated to a temperature of 190°C. over one hour. After confirming that the reaction system is stirred homogeneously, 1.2 parts by weight of dibutyltin oxide is added thereto. The reaction mixture is heated from that temperature to 240°C. over 6 hours, and the dehydration condensation reaction is continued at 240°C. for 4 hours, while distilling water produced, thereby providing a polyester resin having an acid value of 10.0 mgKOH/g, a weight average molecular weight of 12,000 and a glass transition temperature of 60°C.

The polyester resin maintained in a molten state is supplied to an emulsification dispersing device (Cavitron CD1010, available from Eurotec, Ltd.) at a rate of 100 g/min. Diluted aqueous ammonia having a concentration of 0.37% by weight, which is obtained by diluting an aqueous ammonia with ion exchanged water, is put in an aqueous medium tank, and is supplied to Cavitron at a rate of 100 g/min simultaneously with the molten polyester resin. Cavitron is operated at a rotation rate of the rotor of 60 Hz and a pressure of 5 kg/m<sup>2</sup>, thereby providing an amorphous resin particle dispersion having an average particle size of 160 nm, a solid content of 30%, a glass transition temperature of 60°C. and a weight average molecular weight Mw of 12,000.

Preparation of Binder Resin 1  
Octanedioic acid 87 parts by weight  
(available from Wako Pure Chemical Industries, Ltd.)  
Decanediol 87 parts by weight  
5 (available from Wako Pure Chemical Industries, Ltd.)

The aforementioned monomers are charged in a flask, and the mixture is heated to a temperature of 160°C. over one hour. After confirming that the reaction system is stirred homogeneously, 0.02 part by weight of dibutyltin oxide is added thereto. The reaction mixture is heated from that temperature to 200°C. over 6 hours, and the dehydration condensation reaction is continued at 200°C. for 4 hours, while distilling water produced, thereby completing the reaction. The reaction mixture is cooled and then subjected to solid-liquid separation, and the obtained solid content is dried in vacuum at 40°C., thereby providing a binder resin 1.

The obtained binder resin 1 has a melting point of 70°C. as measured with a differential scanning calorimeter (DSC-7, available from Perkin-Elmer, Inc., and a weight average molecular weight of 15,000 as measured with a molecular weight measuring device, HLC-8020, available from Tosoh Corporation, with tetrahydrofuran (THF) as a solvent.

#### Preparation of Crystalline Resin Particle Dispersion

|                                                                                    |                     |
|------------------------------------------------------------------------------------|---------------------|
| Binder resin 1                                                                     | 50 parts by weight  |
| Anionic surfactant<br>(Neogen SC, available from Dai-ichi Kogyo Seiyaku Co., Ltd.) | 2 parts by weight   |
| Ion exchanged water                                                                | 200 parts by weight |

The aforementioned components are heated to 120°C., sufficiently dispersed with Ultra-Turrax, available from IKA Works, Inc., and then dispersed with a pressure discharge homogenizer, and the solid content is recovered when the volume average particle size becomes 180 nm. Thus, a crystalline resin particle dispersion having a solid content of 20% is obtained.

#### Toner 2

|                                       |                     |
|---------------------------------------|---------------------|
| Amorphous resin particle dispersion   | 150 parts by weight |
| Colorant particle dispersion          | 30 parts by weight  |
| Releasing agent particle dispersion 1 | 40 parts by weight  |
| Crystalline resin particle dispersion | 50 parts by weight  |
| Polyaluminum chloride                 | 0.4 part by weight  |

The aforementioned components are sufficiently mixed and dispersed with Ultra-Turrax, available from IKA Works, Inc., in a stainless steel flask, and then heated to 48°C. under stirring over a heating oil bath. After maintaining at 48°C. for 60 minutes, 70 parts by weight of the same resin particle dispersion as above is slowly added thereto.

Thereafter, the pH inside the system is controlled to 8.0 with a sodium hydroxide aqueous solution having a concentration of 0.5 mol/L, and the reaction mixture is heated to 90°C. and maintained for 3 hours under continuously stirring with the stainless steel flask being sealed and the stirrer shaft being sealed with a magnetic seal. After completing the reaction, the reaction mixture is cooled at a temperature decreasing rate of 2°C. per minute and then filtered. The solid content is sufficiently rinsed with ion exchanged water, and then collected by solid-liquid separation by Nutsche suction filtration. The solid content is again dispersed in 3,000 parts by weight of ion exchanged water at 40°C. and stirred and rinsed at 300 rpm for 15 minutes. The rinsing operation is repeated five times, and when the pH of the filtrate becomes 6.5 and the electroconductivity thereof becomes 6.5  $\mu$ S/cm, the solid

content is collected by solid-liquid separation by Nutsche suction filtration with No. 5A filter paper. The solid content is continuously dried under vacuum for 12 hours to provide toner mother particles.

The toner mother particles has a volume average particle size  $D_{50v}$  of 6.3  $\mu\text{m}$  and a volume average particle size distribution index GSD $v$  of 1.20, as measured with Coulter Counter TA-II (available from Beckman Coulter, Inc.). The shape of the mother particles is observed with Luzex image analyzer (available from Nireco Corporation), and as a result, the particles have a shape factor SF1 of 135, which shows a potato-like shape. The glass transition temperature of the toner mother particles is 52° C. To the toner mother particles, silica ( $\text{SiO}_2$ ) fine particles having an average primary particle size of 40 nm having been subjected to a surface hydrophobic treatment with hexamethylsilazane and metatitanic acid compound fine particles having an average primary particle size of 20 nm, which are a reaction product of metatitanic acid and isobutyltrimethoxysilane, are added to make a coverage of 40% with respect to the surface of the colored particles, followed by mixing with a Henschel mixer, thereby providing a toner.

#### Example 1

The toner 1 and the carrier 1 are mixed to make a ratio of the toner of 8% by weight, thereby providing a developer 1.

#### Examples 2 to 9 and Comparative Example 1 to 6

Developers 2 to 9 and C1 to C6 are prepared in the same manner as in Example 1 except that the toners and the carriers shown in Table 1 are used.

#### Evaluation of Reproducibility of Thin Lines

The reproducibility of thin lines is evaluated in an environment at a temperature of 28° C. and a humidity of 85% RH in an evaluation room. The paper used for evaluation is A4 paper (P Paper, available from Fuji Xerox Co., Ltd.). The image forming apparatus used for evaluation is a modified machine of ApeosPort-II 400 (available from Fuji Xerox Co., Ltd.) having a trickle developing system, in which the circumferential velocity of the developing sleeve of the developing device is changed to 500 mm/sec.

5,000 sheets of images with an image density of 20% are formed, and then 5,000 sheets of images with an image density of 5% are formed. The image formation is repeated, and 150,000 sheets at most of images are formed. In the image formation, a halftone image containing thin lines drawn at an angle of 45° with respect to the process direction of the developer is formed every 10,000 sheets (including before starting the image formation), and disturbance of the thin lines (the thickness and density of the lines) is confirmed. The evaluation is terminated at the number of sheets when disturbance occurs. Even though disturbance does not occur at 150,000 sheets, the evaluation is not continued any more. The tolerance of the evaluation of reproducibility of thin lines is 100,000 sheets of more.

#### Evaluation of Image Defect

The image defect is evaluated in an environment at a temperature of 10° C. and a humidity of 15% RH in an evaluation room. The paper and the apparatus for evaluation are the same as in the evaluation of reproducibility of thin lines. After forming 10,000 sheets of images with an image density of 5%, an image shown in FIG. 1 is output, and the length  $t$  (mm) of deletion (white dropout) is measured with a loupe equipped with a scale. The tolerance of the evaluation of image defect is a length of deletion of less than 0.5 mm.

The results of the evaluations are shown in Table 1. In Example 9 and Comparative Example 6, the development is performed without trickle development.

TABLE 1

|    | Toner                 | Carrier    | Trickle development | Evaluation of reproducibility of thin lines              |                        | Evaluation of image defect (length of deletion (mm)) |
|----|-----------------------|------------|---------------------|----------------------------------------------------------|------------------------|------------------------------------------------------|
|    |                       |            |                     | (number of sheets when disturbance of thin lines occurs) | (number of thin lines) |                                                      |
| 15 | Example 1 toner 1     | carrier 1  | yes                 | 130,00                                                   | 0.3                    |                                                      |
|    | Example 2 toner 1     | carrier 2  | yes                 | >150,000                                                 | 0.2                    |                                                      |
|    | Example 3 toner 1     | carrier 3  | yes                 | 130,000                                                  | 0.3                    |                                                      |
| 20 | Example 4 toner 1     | carrier 4  | yes                 | 130,000                                                  | 0.4                    |                                                      |
|    | Example 5 toner 1     | carrier 5  | yes                 | 110,000                                                  | 0.2                    |                                                      |
|    | Example 6 toner 1     | carrier 6  | yes                 | 120,000                                                  | 0.4                    |                                                      |
|    | Example 7 toner 1     | carrier 7  | yes                 | >150,000                                                 | 0.3                    |                                                      |
| 25 | Example 8 toner 2     | carrier 1  | yes                 | 140,000                                                  | 0.3                    |                                                      |
|    | Example 9 toner 1     | carrier 1  | no                  | 110,000                                                  | 0.3                    |                                                      |
|    | Comparative 1 toner 1 | carrier 8  | yes                 | 70,000                                                   | 0.6                    |                                                      |
| 30 | Comparative 2 toner 1 | carrier 9  | yes                 | 80,000                                                   | 0.7                    |                                                      |
|    | Comparative 3 toner 1 | carrier 10 | yes                 | 100,000                                                  | 1.0                    |                                                      |
| 35 | Comparative 4 toner 1 | carrier 11 | yes                 | 30,000                                                   | 0.4                    |                                                      |
|    | Comparative 5 toner 2 | carrier 8  | yes                 | 60,000                                                   | 0.6                    |                                                      |
| 40 | Comparative 6 toner 1 | carrier 8  | no                  | 50,000                                                   | 0.6                    |                                                      |
|    | Example 6             |            |                     |                                                          |                        |                                                      |

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention defined by the following claims and their equivalents.

What is claimed is:

1. A carrier for developing an electrostatic image, comprising:  
magnetic core material particles; and  
a coated layer coated on the magnetic core material particles,  
the coated layer containing a resin having a monomer unit represented by following formula (A'):



wherein:

R<sup>1</sup> represents a hydrogen atom or a methyl group;  
 R<sup>2</sup> represents a hydrogen atom, an alkyl group, an aryl group or an aralkyl group;  
 R<sup>6</sup> represents an alkyl group;  
 R<sup>7</sup> to R<sup>9</sup> each independently represent a hydrogen atom or an alkyl group;  
 R<sup>10</sup> represents an alkyl group, an aryl group, or an aralkyl group;  
 L<sup>1</sup> represents a single bond or an alkylene group; and content of the monomer unit represented by the formula (A') is 10% by mol or more.

2. The carrier for developing an electrostatic image according to claim 1, wherein the coated layer contains carbon black.

3. The carrier for developing an electrostatic image according to claim 2, wherein a content of the carbon black in the

coated layer is approximately 15.0% by mass or less based on the resin having a monomer unit represented by the formula (A').

4. The carrier for developing an electrostatic image according to claim 1, wherein in the formula (A'), R<sup>2</sup> represents a hydrogen atom or an alkyl group having from 1 to 4 carbon atoms.

5. A developer for an electrostatic image, comprising: the carrier for developing an electrostatic image according to claim 1, and a toner.

6. The developer for an electrostatic image according to claim 5, wherein the toner contains a crystalline resin.

7. An image forming method comprising: charging an image holding member; exposing a surface of the image holding member, thereby forming an electrostatic latent image; developing the electrostatic latent image formed on the surface of the image holding member, with a two-component developer, thereby forming a toner image; transferring the toner image formed on the surface of the image holding member, to a surface of a transfer material; and fixing the toner image transferred to the transfer material, wherein the two-component developer is the developer for an electrostatic image according to claim 5.

8. The carrier for developing an electrostatic image according to claim 1, wherein content of the monomer unit represented by the formula (A') is 20% by mol or more.

9. The carrier for developing an electrostatic image according to claim 8, wherein content of the monomer unit represented by the formula (A') is 30% by mol or more.

\* \* \* \* \*